# EUROPEAN PATENT SPECIFICATION

(11) **EP 0 558 205 B1**
(45) Date of publication and mention of the grant of the patent: **06.08.1997**
(21) Application number: 93300982.1
(22) Date of filing: 11.02.1993
(51) Int. Cl.: D04H 1/70

(54) **Method for corrugated bonded or thermo-bonded fiberfill and structure thereof**
Verfahren zum Wellen und zum Verbinden oder thermischen Verbinden von Füllmaterial und dadurch hergestelltes Füllmaterial.
Méthode pour onduler et lier ou lier thermiquement un garnissage fibreuse et sa structure

(30) Priority: 26.02.1992 US 841805
(43) Date of publication of application: 01.09.1993
(73) Proprietor: CHIEN, Jung-Fu, Lin 1, Ching Hu Village, Lin Kou Hsiang, Taipei Hsien (TW)
(72) Inventor: Chien, Tien Sheng, (TW)
(74) Representative: Harvey, David Gareth

(56) References cited:
- EP-A- 0 350 627
- FR-A- 2 117 703
- US-A- 2 454 175
- US-A- 4 129 675
- US-A- 4 576 853

## Description

The present invention relates to a method for corrugating bonded fiberfill, especially to a resin-bonded or thermo-bonded fiberfill structure formed therefrom.

According to prior art as shown in Fig. 1, after opening bale and carding fiber to a web A, the web A is shaped into criss-cross laminations A' to create strength in both longitudinal and transverse directions. This is accomplished by sequential conveying belts B, C, and D, which transversely convey the web A. Belt E conveys longitudinally, whereas conveying belts C and D independently move to and fro transversely. After the criss-cross lamination A' is shaped by cross lapping, resin is sprayed on the criss-cross lamination A', thereby penetrating and bonding the lamination A'. However, the prior process possesses the following drawbacks:
1. The thickness of the web A' needs to be diversified for various applications. The thickness of the lamination A' depends on the number of single webs A, i.e., the manufacturing conditions must be controlled under a higher conveying speed of conveying belts B, C, and D; a higher transverse moving speed of conveying belts of C and D; and/or a lower speed of conveying belt E. Regarding a specification of 500g/cm² of the bonded fiberfill, the cross angle of lamination A' ends up being small or even nearly zero, thereby maintaining transverse strength but, at the same time, decreasing longitudinal strength, i.e., the performance of final product is inferior with regard to the longitudinal strength.
2. Taking a carding web of 20g/cm², for example, a final product to the specification of 500g/cm² necessitates 25 layers of web, thereby resulting in low productivity, poor resin-penetration, and difficulty in ensuring the criss-cross lamination A' bonds together.
3. Conventional resin-bonded fiberfill only exhibits strength in transverse and longitudinal directions but lacks three-directional strength; therefore, the final products are poor in anti-compression properties, etc.

It is the purpose of this present invention, therefore, to mitigate and/or obviate the above-mentioned drawback in the manner set forth in the detailed description of the preferred embodiment.

Accordingly, it is an object of this invention to provide a method for corrugating bonded fiberfill which enhances three-directional strength and resilience of the final product.

This invention seeks to provide a method for corrugating bonded fiberfill which allows excellent penetration of resin and hot air by means of resin bonding or thermo bonding, thereby resulting in products having increased strength.

This invention also seeks to provide an improved structure of resin-bonded or thermo-bonded fiberfill which possesses high resistance to compression and high air permeability, for use in quilts, pillows, cushioned seats, cushions, mattresses, sleeping bags, ski jackets, etc. and as filtering material.

Likewise this invention seeks to provide an improved structure of resin-bonded or thermo-bonded fiberfill which can be made available in different thicknesses by regulating the corrugated fiber web, thereby maintaining good anti-compression and air permeability qualities.

The invention will now be explained in more detail, by way of example only, in the following description taken in conjunction with the accompanying drawings in which:
Fig. 1 is a perspective view of a cross-lapping machine according to prior art;
Fig. 2 is a schematic view of an apparatus for corrugating resin-bonded fiberfill according to the present invention;
Fig. 3 is a schematic view of an apparatus for corrugating thermo-bonded fiberfill according to the present invention, optionally with another two outer webs adhering onto the corrugated fiber web;
Fig. 4 is a perspective view of an improved structure of resin-bonded or thermo-bonded fiberfill according to the present invention;
Fig. 5 is a perspective view of an embodiment in accordance with the Fig. 3;
Fig. 6 is a side view of another embodiment in accordance with the present invention, where a fiber web is saw tooth-like; and
Fig. 7 is a side view of yet another embodiment in accordance with present invention, where the fiber web is triangularly corrugated.

Now referring to the drawings, initially to Fig. 2, a preferred embodiment of an apparatus for implementing a method for corrugating resin-bonded or thermo-bonded fiberfill in accordance with the present invention is shown. The method proceeds as follows.

A bale of fiber is initially opened, carded, and formed into a fiber web, which is indicated by reference numeral 40. The fiber web 40 is fed into a cross-lapping machine 10 which laps the fiber web 40 in alternating directions.

After leaving the cross-lapping machine 10, the fiber web 40 is drafted by a drafting machine 15, thereby increasing the longitudinal strength thereof. The fiber web 40 is conveyed between a pair of parallelly-spaced conveyor belts or rollers 20. The conveyor belts or rollers 20 pivot about an axis at the entrance thereto, as shown by the arrows in Fig. 2, so that as the fiber web 40 exits therefrom, the pivoting motion folds the fiber web 40 at the laps formed by the cross-lapping machine 10, forming a corrugated structure as the fiber web 40 enters a conveying passage 30. The conveying passage 30 has a height set at a predetermined height desired of the corrugations of the fiber web 40.

At this point, the fiber web 40 is applied with a first outer web 1 which is conveyed from a first roller 70, and then passes into a spraying machine 50, where resin is sprayed onto one side of the first outer web 1. Then, the fiber web 40 having the first outer web 1 thereon is heated and dried by oven 60. After leaving the oven 60, the fiber web 40 is applied with a second outer web 1 which is conveyed from a second roller 70, and then passes into a spraying machine 80, where resin is sprayed onto the second outer web 1. Again, the fiber web 40 having two outer webs 1 thereon is heated and dried by the oven 60. The resin will adhere the corrugations 21, as shown in Fig. 5. The first and second outer webs 1 can be optionally applied to the fiber web 40 after passing into the spraying machines 50 and 80 respectively. Alternatively, products possessing no sandwich structure, as shown in Fig. 4, can be manufactured by canceling the step of applying the two outer webs 1 on the fiber web 40.

Fig. 4 provides a perspective view of the product having no sandwich structure. The fiber web 40 possess strength along the three directional axes thereof, significantly increasing the strength and resilience of the overall structure. Furthermore, the spaces between the contact sites 41 and 42 of the corrugations allow resin to be uniformly dispersed and penetrated throughout the structure, which subsequently facilitates the drying and curing process.

Instead of adding resin, fiber of low melting point can be blended into regular fiber, and when melted will bond the corrugations and the regular fiber together. Before passing into the oven 60, the fiber web 40 is optionally sandwiched with a pair of transversely-positioned outer webs 1 respectively conveyed from two rollers 70. The sandwich structure passes into the oven 60, thereby bonding the outer webs 1 on the fiber web 40.

Preferably as shown in Fig. 5, corrugations 21 of the fiber web 40 are accordion-like, where top and bottom ends thereof are generally rounded, with respective inner and outer spaces 22 formed between respective corrugations 21 and the outer webs 1. Also, in accordance with the present invention, the corrugations 21 of the fiber web 40 can be saw tooth-shape or triangularly-shaped, as respectively shown in Figs. 6 and 7.

Overall, the structure of the present invention has a high degree of air permeability, resistance to compression, and loftiness, and is useful in quilts, pillows, cushioned seats, cushions, mattresses, sleeping bags, snow clothing, etc. and as filtering material.

While the present invention has been explained in relation to its preferred embodiment, it is to be understood that various modifications thereof will be apparent to those skilled in the art upon reading this specification. Therefore, it is to be understood that the invention disclosed herein is intended to cover all such modifications as shall fail within the scope of the appended claims.

## Claims

1. A method for forming a corrugated, thermo-bonded fiberfill structure comprising the steps of:
(a) adding fiber of low melting point to other fibers;
(b) opening and carding a bale of the fibers of the step (a) to form a fiber web (40);
(c) lapping said fiber web in alternating directions to form alternating laps;
(d) drafting said fiber web, such that the longitudinal strength of said fiber web is increased;
(e) folding said fiber web at said alternating laps to form corrugations (21); and
(f) subjecting the web to conditions such that said fiber of low melting point bonds and maintains said corrugations (21).

2. A method as claimed in claim 1, further comprising a step after said step (e) of applying to said fiber web (40) a transversely-positioned outer web (1), or a pair of outer webs (1) sandwiching said fiber web (40).

3. A corrugated, thermo-bonded fiberfill structure obtainable by the method set forth in claim 1 or claim 2, wherein the corrugations (21) are accordian-shaped, sawtooth shaped or of triangular zig-zag form.

## Patentansprüche

1. Verfahren zum Herstellen einer gewellten, thermisch verbundenen Faserfüllstoffstruktur mit den Schritten:
(a) Hinzufügen einer Faser mit niedrigem Schmelzpunkt zu anderen Fasern;
(b) Öffnen und Kardieren eines Faserballens des Schrittes (a) zum Herstellen ein Faserbahn (40);
(c) Übereinanderlegen der Faserbahn in abwechselnden Richtungen zum Herstellen abwechselnder Lagen;
(d) Verstrecken der Faserbahn in der Art, daß die Längsrichtungsfestigkeit erhöht wird;
(e) Falten der Faserbahn bei den abwechselnden Lagen zum Herstellen von Wellungen (21); und
(f) Unterwerfen der Bahn unter Bedingungen der Art, daß die Faser mit dem niedrigen Schmelzpunkt die Wellungen (21) verbindet und aufrechterhält.

2. Verfahren nach Anspruch 1, ferner umfassend einen Schritt nach dem Schritt (e) zum Aufbringen einer querverlaufend angeordneten Außenbahn (1) oder eines Paares von Außenbahnen (1), welche die Faserbahn (40) einschließen.

3. Gewellte, thermisch verbundene Faserfüllstoffstruktur, erhältlich durch das in Anspruch 1 oder Anspruch 2 beschriebene Verfahren, wobei die Wellungen (21) Akkordeonartig, Sägezahn-artig oder von dreieckiger Zick-Zack-Form sind.

## Revendications

1. Procédé pour former une structure à garnissage fibreux liée thermiquement et ondulée comprenant les étapes consistant à :
(a) ajouter une fibre de bas point de fusion à d'autres fibres,
(b) ouvrir et carder une balle des fibres de l'étape (a) pour former un tissu de fibres (40),
(c) enrouler ledit tissu de fibres dans des directions alternées pour former des enroulements alternés,
(d) étirer ledit tissu de fibres de telle manière que la résistance longitudinale dudit tissu de fibres soit accrue,
(e) plier ledit tissu de fibres au niveau desdits enroulements alternés pour former des ondulations (21), et
(f) soumettre le tissu à des conditions telles que ladite fibre de bas point de fusion lie et maintienne lesdites ondulations (21).

2. Procédé selon la revendication 1, comprenant en outre une étape après l'étape (e) consistant à appliquer audit tissu de fibres (40) un tissu extérieur disposé transversalement (1), ou une paire de tissus extérieurs (1) entourant en une configuration sandwich ledit tissu de fibres (40).

3. Une structure à garnissage fibreux liée thermiquement et ondulée obtenue par le procédé défini dans la revendication 1 ou 2, dans lequel les ondulations (21) sont en forme d'accordéon, en forme de dent de scie ou en forme de zig-zag triangulaire.
